

# UNITED STATES PATENT OFFICE.

SUMNER SIMPSON, OF BRIDGEPORT, CONNECTICUT, ASSIGNOR TO THE RAYBESTOS CO., OF BRIDGEPORT, CONNECTICUT, A CORPORATION OF CONNECTICUT.

## CLUTCH-FACING.

1,270,559.

Specification of Letters Patent. Patented June 25, 1918.

No Drawing.

Application filed September 19, 1917. Serial No. 192,232.

To all whom it may concern:

Be it known that I, SUMNER SIMPSON, a citizen of the United States, residing in the city of Bridgeport, county of Fairfield, and 5 State of Connecticut, have invented certain new and useful Improvements in Clutch-Facings, of which the following is a specification.

This invention relates to improvements in 10 clutch facings and process of making same and refers more particularly to a clutch facing adapted for use in motor vehicles and the like.

Among the salient objects of the present 15 invention are to provide a clutch facing which can be made from unwoven felted asbestos fiber, the fiber being united into a compact, substantially homogeneous and uniform mass, primarily by means of a com- 20 minuted binder; to provide a product of the character referred to, which is uniform in character and uniform in density throughout its wearing surface and to a substantial depth of the latter; to provide a product, the 25 essential body portion of which may be made of short asbestos fiber united through the medium of a comminuted binder; to produce a product of the above character which can be formed to micrometer measurements, both as regards its width and thickness; to provide a product having the required co-efficient of friction, which has a maximum wearing resistance and is capable of withstanding high temperatures without 30 physical or chemical change; to provide a product which can be made of unspun short fiber, to which may be added the dust or screenings of said fiber, united and held into a compact and relatively solid mass, sub- 35 stantially by the binding action of a material, comminuted or granular when dry; to provide a preformed asbestos or other suitable fibrous sheet which may be formed out of unwoven felted short fiber and out of 40 which the facings may be stamped or cut either before or after saturation of the sheet with the binder; to provide a process of making the above product which eliminates the expensive and numerous operations neces- 45 sary in making a woven facing and which permits of the use of the cheapest portion of the fiber, which forms a product having a uniform character and density, not possible in the fibrous facings of the prior art; to 50 provide a process in which the material left

after cutting or stamping out the facings can be re-treated to make a new sheet, thus reducing the waste material to a minimum; and in general to provide an improved product and process of the character referred to. 60

In friction facings, for motor vehicles, and the like, the following are desirable, if not essential, characteristics which should be inherent in a good friction facing.

1. The co-efficient of friction should be 65 sufficiently high to meet all requirements.

2. The facing should have a high wear re- 70 sisting and heat resisting ability.

3. The facing should be of uniform char- 75 acter and density so that even if the exposed surface wears away, there will be at all times a uniform wearing surface.

4. The facing should be as free as possible 80 from fibers which serve only as binders and are not themselves capable of standing abra- 75 sion or heat such as cotton, hemp or sisal fibers and paper.

5. It is desirable to use as many short 85 fibers as possible for the reason that the long fibers are relatively expensive.

6. The margin of profit makes it exceed- 90 ingly advantageous to have the process as economical and simple as possible.

7. The waste stock should be reduced to a 95 minimum.

8. The facing should be a tough, compact mass, free from any tendency to cause a separation of its component parts and free of any tendency to ravel.

9. The facing should be capable of being 90 punched, or drilled and countersunk for rivet holes without destroying its efficiency.

Asbestos from the mine run consists of 95 relatively long fibers, known in the art as crude asbestos and relatively short fibers, known in the art as fiber asbestos. The crude asbestos is the only portion that can be utilized for spinning and weaving; the fiber asbestos cannot be used for such purpose and accordingly low grade fiber asbestos has 100 never been utilized in the manufacture of woven clutch facing. Heretofore, no asbestos clutch facing has been successfully made except from woven fiber.

By means of the present invention, the 105 low grade asbestos fibers or short fibers can be utilized to form the essential body portion of the clutch facing as heretofore stated. These fibers after being felted are perma- 110 nently united into a compact uniform mass

by means of a comminuted binder carried during the process of manufacture in a suitable liquid vehicle.

One illustration of the manner in which the process may be carried out is as follows: The asbestos fiber or low grade short fiber as it comes from the mine is first ground in a suitable grinding machine or crusher.

This ground material is then put into a beater, mixed with water or other liquid solution and beaten into a pulp. The wet pulp is then delivered to a paper making machine and formed into laminated sheets of suitable width and thickness. From there the sheet passes through suitable presses and driers.

Preferably, this sheet is of sufficient width to permit of five or more clutch facings to be stamped or cut out of its width, although the sheet may be made of any width suitable for meeting the particular requirements. Either before or during the operation of cutting the sheet is pressed to proper sheets. Where clutch facings of the ring type is to be made, they can be stamped or cut out of the body of the sheet forming an endless annular or ring member. By making these clutch facings in the form of an endless ring, the difficulties or objections incident to a jointed woven ring are obviated. Clutch facings of the cone type can also be formed from the sheet by cutting out segments to the radius of the cone and then forming them into proper shape. Where endless ring shaped facings are cut out of this sheet of abnormal width, a large part of the sheet is necessarily left from which no further rings can be formed. This otherwise waste material is saved by putting it back into the grinder and beater and running it through the process as a new batch.

The clutch facings are next impregnated or saturated in suitable dipping tanks with a binder. This binder may consist of either a suitable vegetable oil or gum, or mineral oil and gum, or bitumens, or a combination of the same, the comminuted solid matter

being carried in a suitable vehicle, such as benzine, benzene, coal tar naphtha, petroleum naphtha, alcohol, or amyl acetate or the like which also serves as a solvent. It is of course, desirable, that the binder have adhesive properties so as to more firmly unite the asbestos fiber into a compact substantially homogeneous and uniform mass.

50  
55

The saturated or impregnated material is then put into a drying oven, which may be heated by closed steam coils or otherwise, preferably to a temperature not in excess of 200° F., which drying step drives out the solvent. After treating the product is put into a curing oven, where it is subjected to a higher heat, for example, from 250 to 500° F., more or less. This step gives the necessary hardness to the fabric or facing.

60  
65

The invention is not limited to the details of product and process here described, except as set forth in the appended claims.

I claim as my invention:

1. A clutch facing having a wearing surface of uniform character and density throughout a substantial depth, the essential body portion of said wearing surface being formed of unwoven felted short asbestos fiber, and a comminuted adhesive binder 70 permanently uniting the fiber into a solid compact mass.

75

2. A friction facing having a compressed wearing surface, of uniform density throughout a substantial depth, the essential body portion of said wearing surface being formed of unwoven felted fiber having a high abrasive resisting character and a binder permanently uniting the fiber.

80

3. A clutch facing blank of abnormal width, the essential body portion of which consists of a sheet of unwoven felted asbestos fiber adapted to be formed into a plurality of facings and capable of being permanently united into a solid compact mass 90 by intimately uniting the fiber with a comminuted adhesive binder.

85

SUMNER SIMPSON.

## DISCLAIMER.

1,270,559.—*Sumner Simpson*, Bridgeport, Conn. CLUTCH FACING. Patent dated June 25, 1918. Disclaimer filed October 3, 1923, by the assignee, *The Raybestos Company*.

Hereby disclaim the article defined by said claim 2, except when such article is in the form of a relatively thin disk, or plate, or strip, a side, or relatively wide face, of which receives the wear, and wherein during its use no binding medium additional to that used in its manufacture need be applied for preventing material disintegration thereof.

[*Official Gazette October 23, 1923.*]